

June 21, 1938.

N. HAYS

2,121,692

METHOD FOR CLOSING CRACKS IN CASTINGS AND THE LIKE

Filed Nov. 23, 1936

*Fig. 1.*



*Fig. 2.*



*Fig. 3.*



*Fig. 4.*



*Fig. 5.*



*Fig. 6.*



*Fig. 7.*



Newell Hays  
INVENTOR  
BY Victor J. Evans & Co.  
ATTORNEYS

## UNITED STATES PATENT OFFICE

2,121,692

## METHOD FOR CLOSING CRACKS IN CASTINGS AND THE LIKE

Newell Hays, El Paso, Tex.

Application November 23, 1936, Serial No. 112,390

## 1. Claim. (Cl. 29—148)

The object of the invention is to provide a method whereby, without the use of heat, cracks in a metal casting may be effectively closed; and to provide a method for the purpose indicated which may be carried out with the expenditure of a minimum of time and which will require no particular skill on the part of the operator.

With this object in view, the invention consists of certain steps to be successively performed, as illustrated in the accompanying drawing, wherein:

Figure 1 is a plan view of a portion of the casting containing a crack in which the first step in the method has been performed.

Figure 2 is a plan view of the casting following the performance of the second step.

Figure 3 is a plan view of the casting after the performance of the third or final step.

Figure 4 is a sectional view on the plane indicated by the line 4—4 of Figure 1.

Figure 5 is a sectional view on the plane indicated by the line 5—5 of Figure 2.

Figures 6 and 7 are sectional views on the planes indicated by the lines 6—6 and 7—7 respectively of Figure 3.

In carrying out the improved method, let the casting or other metal part 10 be one in which a crack, such as that indicated at 11, has occurred. A series of holes 12 will be drilled along a line generally following the line of the crack, the holes being uniformly spaced with a pitch between centers slightly in excess of the diameters of the holes. Then the casting will be channeled on the outer surface, as indicated at 13, so that the holes will be disposed within the

channel. The holes are then tapped, as indicated at 14, a comparatively fine pitch of thread being preferably used.

The next step is the plugging of the holes which is accomplished by means of the insertion of screws 15 which may be and preferably are in the form of blind set screws, although headed screws may be employed in some cases which of course will call for wider spacing between adjacent screws than in the preferred plan of carrying out the method.

After the holes have been plugged with the screws, as shown in Figure 5, the outer ends are peened over or beaten down into the channel 13, so that the metal completely fills the latter, 15 as shown in Figures 3, 6 and 7, any excess metal being cleaned off with a suitable dressing tool, such as a file, emery wheel, or the like.

In this way, the crack will not only be completely closed but the repair will be hardly noticeable, if the work is carefully done, as it may be with a minimum of skill required on the part of the operator.

The invention having been described, what is claimed as new and useful is:

A method for closing cracks in castings and the like which comprises drilling spaced holes in the casting in a line generally along the line of the crack, channeling the face of the casting to dispose the holes along the center line of the channel, tapping said holes, inserting screws in the holes, and finally peening over the extremities of the screws to completely fill the channel with the metal thereof.

NEWELL HAYS. 35